

## UNITED STATES PATENT OFFICE

2,272,063

## ELECTRIC CONTACTING MEMBER

Franz R. Hensel and Kenneth L. Emmert, Indianapolis, Ind., assignors to P. R. Mallory & Co., Inc., Indianapolis, Ind., a corporation of Delaware

No Drawing. Application June 5, 1939,  
Serial No. 277,496

3 Claims. (Cl. 200—166)

This invention relates to electric contacts.

An object of the invention is to improve the characteristics of an electrical contacting element containing silver.

Another object of the invention is to provide a silver base contact material which will retain a low contact resistance.

A still further object is to provide a new contact material which can be used under severe electrical conditions, without welding.

Other objects of the invention will be apparent from the following description, taken in connection with the appended claims.

The present invention relates to an electric contact and the combination of elements therefore, methods of manufacture and the product thereof, brought out and exemplified in the disclosure hereinafter set forth, the scope of the invention being indicated in the appended claims.

While a preferred embodiment of the invention is described herein, it is contemplated that considerable variation may be made in the method of procedure and the combination of elements, without departing from the spirit of the invention.

The present invention comprises an improvement in silver electric contact elements. According to the invention, the contacts are improved by the addition of beryllium.

The contacts may be composed of silver and beryllium accordingly. The ingredients may be present in approximately the following proportions:

|           |                   |          |
|-----------|-------------------|----------|
| Beryllium | Percent by weight | .05 to 4 |
| Silver    | Balance           |          |

One of the experimental alloys, containing .94% beryllium, had a conductivity in the as cast condition of 67.2%, a hardness in the as cast condition of 43 Rockwell F, which increased to 87 Rockwell F, after 25% cold swaging. The specific gravity of this material was 10.12 grams per c. c., as compared to 10.5 grams per c. c. for fine silver. The beryllium has a much lower specific gravity than fine silver and therefore the addition of beryllium lowers the density of the finished alloy, which is of considerable commercial importance, because it is possible to obtain a larger number of finished pieces, and more particularly finished contacts, per unit weight. In most constitutional diagrams the percentages are given by weight percentages. A much clearer picture, however, can be obtained, if the atomic percentages are used, because there is an enormous difference in the atomic weights of silver

and beryllium, silver being 108, and beryllium 9.

In order to avoid segregation during melting, a master alloy was used containing 4 to 6% of beryllium. No difficulty was encountered in melting and pouring these alloys. It was found advisable, in certain cases to add a flux which consisted of sodium fluoride and beryllium fluoride.

The addition of small percentages to silver causes a very marked decrease in the freezing point, the liquidus curve falling steeply, until a beryllium content of .97 is reached. This corresponds to an atomic percentage of 10.4 beryllium. The melting point of the eutectic is 881 degrees C. With increasing beryllium, the liquidus first rises very sharply, then flattens out. It was found that the maximum solid solubility was 3.5 atomic percent of beryllium at the temperature of the freezing point of the eutectic. The solubility decreases slowly with decreasing temperature. This indicated that the materials can be improved slightly by age hardening, which can be obtained by a heat treatment of the alloys, consisting usually in a quenching operation and a subsequent aging operation. It was possible to raise both the hardness of the material and the electrical conductivity. Under the microscope, the material containing 10.4 atomic percent of beryllium, shows a typical structure of an eutectic, the matrix consisting of silver and a free constituent consisting of the beryllium rich solid solution. In the preparation of the alloys it has also been found of advantage to add materials which are very powerful deoxidizers and degasifiers, such as, for instance, lithium. Alloys produced in such a manner are free from beryllium oxide and therefore show improved ductility, impact strength and if used as an electrical contact, show a decreased tendency to transfer.

Silver-beryllium alloys lend themselves very readily to be prepared in the form of contacts from either swaged material, drawn wire or rolled sheet. Silver-beryllium alloys lend themselves also very readily to be prepared in the form of contact bimetals in which one side consists of a base metal, such as an alloy of iron, or nickel, or a copper base material and a silver-beryllium material on the other side. An alloy of the eutectic composition containing .94 weight percent of beryllium was tested in a standard critical current test. In this test, contacts of similar physical dimensions are studied on a resistive, inductive circuit at 470 cycles per minute, and wherein current flowing in the circuit was increased periodically to obtain the definite current values, in

comparison with contact materials produced in the prior art. The alloy tested gave a critical current of 15 amps. and a negative transfer of 0.15. It was found that by increasing the beryllium content, a peak was reached in which the critical current was a maximum and the transfer, a minimum. The peak was located between a beryllium content of about 1 to 3%.

It was found that after completing the tests, the material retained an abnormally low contact resistance, the eutectic material retained an abnormally low contact resistance, the eutectic material showing a contact resistance of only .05 milliohm, after 30,000 cycles. This is considerably below coin silver, standard silver and even fine silver.

The alloy of the present invention has been found useful for a large number of electric contact applications, such as for instance, sensitive direct current relays, overload cutouts, voltage regulators, thermostats, indicating and recording gauges, and the like.

The alloys of the present invention have been found to have excellent free machining properties for the production of commercial parts where

high speed production and corrosion resistance are required.

While the present invention as to its objects and advantages has been described herein as carried out in specific embodiments thereof, it is not desired to be limited thereby, but it is intended to cover the invention broadly, within the spirit and scope of the appended claims.

What is claimed is:

- 10 1. An electric contact element consisting of .05 to 4% beryllium by weight and the balance silver.
2. An electric contact member comprising a bimetal consisting of a base metal backing and a facing of an alloy of .05 to 4% beryllium by weight and the balance silver.
- 15 3. An electric contact element consisting of silver-beryllium eutectic containing substantially 10.4 atomic percent of beryllium and the balance silver, said contact element being characterized by low specific resistance, low contact resistance and low tendency to weld in service.

FRANZ R. HENSEL.  
KENNETH L. EMMERT.